

## UNITED STATES PATENT OFFICE

2,453,816

RUST PREVENTIVE SLUSHING COMPOUND  
FOR CARTRIDGE CLIPSHans Schindler, Evanston, and Paul T. Anderson,  
Park Ridge, Ill., assignors to The Pure Oil Company,  
Chicago, Ill., a corporation of OhioNo Drawing. Application July 10, 1944.  
Serial No. 544,328

4 Claims. (Cl. 106—14)

1

This invention relates to slushing oils and more particularly to slushing oils suitable for preventing rusting of metal articles such as cartridge clips, shells and other ordnance goods.

The object of this invention is to provide an effective rust preventing slushing compound for "Parkerized" cartridge clips and other ordnance goods.

We have discovered that a highly effective rust preventing slushing compound can be prepared by saponifying wool grease with litharge to make a lead wool grease soap having a neutralization number between 2.5-4 and preferably approximately 3 and mixing the lead wool grease soap with a light lubricating oil and wetting agent and a thinner in proper proportions.

In preparing our slushing compound, ordinary wool grease, degras or lanolin is mixed with sufficient litharge to produce a soap having a neutralization number of 2.5-4 when completed and preferably around 3. The wool grease and the litharge are heated to a temperature of approximately 350° F. for a period of three hours with agitation in order to complete the saponification.

The finished hot soap is mixed with a low viscosity mineral lubricating oil, preferably one having a viscosity from 60 to 150 seconds Saybolt at 100° F. From 15 to 30 parts by weight of lead-wool grease soap may be mixed with from 30 to 50 parts by weight of the lubricating oil and these figures represent the percentages of these ingredients in the final composition. A wetting agent such as dioctyl ester of sodium sulfo-succinic acid is added to the mixture in amounts such that it is present in the mixture to the extent of 1 to 3%. Any higher alcohol ester of an alkali metal sulfo-succinic acid may be used in place of the dioctyl ester and preferably esters of alcohols having from 8 to 18 carbon atoms in the molecule.

The composition, made as above described, has a semi-solid or greasy texture. This material is thinned with a hydrocarbon solvent having a boiling range up to about 400° F., such as Stoddard solvent, to the extent desired which will depend on the thickness of the film required on the coated object. Any light hydrocarbon solvent having a flash point above 100° F. may be used.

The following composition prepared in accordance with our invention passed the United States

2

Ordnance specification for slushing compound for "Parkerized" cartridge clips.

|                                                                           | Percent by weight |
|---------------------------------------------------------------------------|-------------------|
| Common wool grease                                                        | 17.3              |
| Litharge                                                                  | 3.5               |
| Dioctyl ester of sodium sulfo-succinic acid                               | 2.0               |
| Pennsylvania Neutral having a viscosity of 100 seconds Saybolt at 100° F. | 49.1              |
| Stoddard Solvent                                                          | 28.1              |

The slushing oil is generally applied to the objects to be coated by running the objects in the oil and centrifuging the object to remove excess slushing compound. A thin, greasy or semi-solid film remains on the object after the thinning solvent evaporates which protects the object against rusting.

Although in the formula above set forth the amount of Stoddard solvent is 28.1%, the amount of solvent may be more or less, depending on the thickness of the film it is desired to leave on the coated object. Where a heavy film is desired, the amount of the solvent is low. Where a light film is desired, the amount of the solvent is high.

By following the procedure above set forth in the preparation of the compound, and by adhering to the quantities of the several ingredients previously set forth, a highly useful and effective slushing oil is produced.

We claim:

1. A slushing oil composition consisting of from 15-30% by weight of lead-wool grease soap having a neutralization number of about 3, from 30-50% by weight of mineral oil having a viscosity at 100° F. of from 60 to 150 seconds Saybolt, from 1-3% by weight of a higher alcohol ester of an alkali metal sulfo-succinic acid and the balance a low-boiling hydrocarbon liquid having a flash point of at least 100° F.
2. A slushing oil in accordance with claim 1 in which the ester is dioctyl ester of sodium sulfo-succinic acid and the low-boiling hydrocarbon is Stoddard solvent.
3. A slushing oil consisting of the following substances in approximately the following parts by weight: wool grease—17.3; litharge—3.5; dioctyl ester of sodium sulfo-succinic acid—2; Pennsylvania neutral mineral oil having a viscosity of 100 seconds Saybolt at 100° F.—49.1; Stod-

dard solvent—28.1, and in which the ltharge and wool grease are combined to form a lead-wool grease soap having a neutralization number of about 3.

4. A slushing oil consisting of 30 to 50 per cent by weight of light mineral lubricating oil, 15 to 30 per cent by weight of lead-wool grease soap having a neutralization number of about 3, from 1-3 per cent by weight of a higher alcohol ester of an alkali metal sulfo-succinic acid, and the balance a low-boiling hydrocarbon liquid having a flash point above 100° F.

HANS SCHINDLER.  
PAUL T. ANDERSON.

## REFERENCES CITED

The following references are of record in the file of this patent:

## UNITED STATES PATENTS

| Number    | Name          | Date          |
|-----------|---------------|---------------|
| 620,899   | Ekenberg      | Mar. 14, 1899 |
| 1,364,134 | Morgan        | Jan. 4, 1941  |
| 2,342,027 | Waugh         | Feb. 15, 1944 |
| 2,348,715 | Adams et al.  | May 16, 1944  |
| 2,357,276 | Wachter       | Aug. 29, 1944 |
| 2,392,102 | Ruedrich      | Jan. 1, 1946  |
| 2,418,075 | Kollen et al. | Mar. 25, 1947 |

## FOREIGN PATENTS

| Country       | Date          |
|---------------|---------------|
| Great Britain | May 18, 1921  |
| Great Britain | June 14, 1939 |